

# United States Patent [19]

Liebermann et al.

[11] 4,281,706

[45] Aug. 4, 1981

[54] **METHOD OF MAKING HELICAL METALLIC RIBBON FOR CONTINUOUS EDGE WINDING APPLICATIONS**

[75] Inventors: **Howard H. Liebermann, Schenectady; Peter G. Frischmann, Scotia, both of N.Y.; George M. Rosenberry, Jr., Hendersonville, Tenn.**

[73] Assignee: **General Electric Company, Schenectady, N.Y.**

[21] Appl. No.: **972,240**

[22] Filed: **Dec. 22, 1978**

[51] Int. Cl.<sup>3</sup> ..... **B22D 11/06**

[52] U.S. Cl. ..... **164/463; 164/423**

[58] Field of Search ..... **164/82, 423**

[56] **References Cited**

**U.S. PATENT DOCUMENTS**

989,075 4/1911 Staples ..... 164/423  
2,825,108 3/1958 Pond ..... 164/82

|           |         |                        |           |
|-----------|---------|------------------------|-----------|
| 2,910,744 | 11/1959 | Pond .....             | 164/423 X |
| 3,188,505 | 6/1965  | Wiley .....            | 310/259   |
| 3,674,084 | 7/1972  | Paliwoda .....         | 164/271   |
| 4,155,397 | 5/1979  | Honsinger et al. ..... | 164/423 X |
| 4,187,441 | 2/1980  | Oney .....             | 310/112   |
| 4,211,944 | 7/1980  | Haller .....           | 310/72    |
| 4,211,957 | 7/1980  | Alley et al. .....     | 315/276   |

**FOREIGN PATENT DOCUMENTS**

904048 2/1945 France .....

Primary Examiner—Robert D. Baldwin  
Attorney, Agent, or Firm—Stephen S. Strunck; James C. Davis, Jr.; Leo I. MaLossi

[57] **ABSTRACT**

Metallic ribbon is fabricated in continuous helical form by directing a melt stream or jet onto a rapidly moving substrate surface. The axis of the crucible along which the melt stream or jet is cast is defined by an inverted cone with apex at the point of crucible axis intersection with the substrate surface.

**15 Claims, 10 Drawing Figures**







FIG. 6



FIG. 7

FIG. 8



FIG. 9



**METHOD OF MAKING HELICAL METALLIC RIBBON FOR CONTINUOUS EDGE WINDING APPLICATIONS**

**CROSS-REFERENCE TO RELATED APPLICATION**

This invention is related to the invention disclosed and claimed in copending application Ser. No. 972,239, filed Dec. 22, 1978, in the names of the same inventive entity as the instant application, assigned to the same assignee as the instant application, and entitled "Helical Metallic Ribbon for Continuous Edge Winding Applications".

**BACKGROUND OF THE INVENTION**

**1. Field of the Invention**

This invention relates to a method for making metallic ribbons in helical form for continuous edge winding applications.

**2. Description of the Prior Art**

The fabrication of glassy alloy magnetic ribbon for use in electric motor applications is commonly believed to involve conventional punching operations performed on sheets or strips of the ribbon. However, a low filling or packing factor will result from conventional or prior art laminations of known glassy alloys because of the greater number of punchings required when compared with the number of punchings required when using prior art materials for laminations. This is because of the inherent limit on thickness in melt-quenched glassy alloy specimens. The overall effect is to increase the size and cost of the finished electric motor, thereby negating the savings offered by use of the glassy alloy material. A prior art method of making glassy alloy ribbon is to extrude the alloy in molten form through an appropriate orifice in a crucible and to subsequently impinge the melt jet onto the circumferential surface of a rapidly rotating substrate wheel. The melt jet is typically made to lie parallel to the plane of the substrate wheel. The ribbon so formed has the shape of conventional tape or ribbon and can be wound upon a spool.

It would be desirable to manufacture a motor stator comprising two concentric pieces of material. A center piece would be prefabricated with teeth and windings. The outer piece would be prefabricated or built in situ from an edge-wound strip in the form of a large helix.

Therefore, it is an object of this invention to provide a method for making metallic ribbon in a continuous helical form.

Another object of this invention is to provide a method for making a new and improved edge-wound glassy alloy magnetic ribbon in a helical form.

A further object of this invention is to provide a method for making edge-wound metallic or glassy alloy magnetic ribbon in a nest helical form.

A still further object of this invention is to provide a method for making edge-wound metallic or glassy alloy magnetic ribbon with prefabricated cutouts therein for making, as an example, a motor stator.

Other objects of this invention will, in part be obvious and will, in part, appear hereinafter.

**BRIEF DESCRIPTION OF THE INVENTION**

In accordance with the teaching of this invention there is provided a method for making metallic and glassy alloy ribbons in helical form by chill block melt-spinning. The method includes the process steps of

causing a substrate wheel to rotate at a predetermined speed to impart to a substrate surface thereon a predetermined velocity of from about 12 meters per second to about 50 meters per second. The substrate surface generally is oriented normal to the axis of rotation of the substrate wheel. Molten alloy is formed in a crucible and is extruded through an orifice in the crucible to form a melt stream or jet having a preferred velocity of from about 1 meter per second to about 10 meters per second.

The crucible, the orifice and the melt stream or jet have colinear axes. The crucible axis is positioned on an inverted cone in space above the moving substrate surface and intersects the apex of the cone. The position of the crucible axis on the inverted cone is defined by an inclination angle  $\alpha$  and an azimuthal angle  $\gamma$  having values  $0 \leq |\gamma| \leq 180^\circ$ . The axis of the melt stream or jet lies in a plane defined by the tangent to the rotation of the substrate wheel at the point of intersection of the crucible axis and the normal to the moving substrate surface at the same point of intersection. The angle  $\alpha$  has values of  $30^\circ \leq \alpha \leq 90^\circ$  and preferably  $40^\circ \leq \alpha \leq 70^\circ$ .

The molten alloy cast is rapidly quenched on the moving substrate surface to form a continuous length of an edge-wound metallic ribbon having a helical shape, a substantially uniform cross-section, a pair of opposed substantially parallel major surfaces, and inner and outer peripheral edges. The ribbon assumes an inplane curvature defined by the motion of the substrate wheel at the area of melt stream or jet impingement.

Barrier lines may be provided on the moving substrate surface in the form of a continuous geometric pattern. This geometric pattern is oriented on the moving substrate surface so as to provide a means for providing a geometrical pattern of cutouts in either or both or the inner and outer peripheral edges of the ribbon.

Other embodiments of the process include modifying at least a portion of the moving substrate surface to be inclined toward or away from the axis of rotation of the substrate wheel. Casting the molten alloy on the moving inclined substrate surface produces a continuous length of a nested helical metallic ribbon. The composition of the ribbon may be that of a glassy alloy system which may be successfully produced by rapid quenching from the melt. Typical examples of such systems are Fe-B, Fe-B-C, Fe-B-Si, Fe-Ni-B, Cu-Zr, and the like.

**BRIEF DESCRIPTION OF THE DRAWINGS**

FIG. 1 is a schematic view illustrating fabrication of edge-wound metallic ribbon in a helical form.

FIG. 1a is a top planar view of the schematic of FIG. 1 showing the azimuthal orientation of the melt flow axis in relation to the area of stream impingement on the moving substrate surface 22.

FIG. 2 is a partial cross-section schematic view of fabricating a nested edge-wound metallic ribbon in a helical form.

FIG. 3 is a partial cross-section side elevation view of a nested edge-wound metallic ribbon.

FIG. 4 is a partial cross-section schematic view of fabricating nested edge-wound metallic ribbon in a helical form.

FIG. 5 is a partial cross-section side elevation view of a nested edge-wound metallic ribbon.

FIGS. 6, 7 and 8 are schematic views of fabricating an edge-wound metallic ribbon with a continuous pat-

tern of predetermined periodic geometry in either one or both of the inner or the outer peripheral edges of the ribbon.

FIG. 9 is a schematic view of a portion of ribbon illustrating a continuous geometric pattern within the ribbon.

#### DESCRIPTION OF THE INVENTION

Referring now to FIG. 1, there is shown a method of making edge-wound metallic ribbon 10. Within the limits of the present invention, a ribbon is a thin body whose transverse dimensions are very much smaller than its length.

The ribbon 10 is formed by impinging a melt stream or jet 12 onto a moving substrate surface 13 of a substrate wheel 14, rotating about axis 20, by extrusion of the molten alloy through an appropriate orifice 16 of a crucible 18. The axis 15 of the melt stream or jet 12 is made to lie in a plane 26 defined by the tangent to the rotation of the substrate wheel 14 at the point of melt stream or jet axis 15 intersection 24 and by the normal to the local substrate surface 22 at the same point 24. Upon impingement of the melt stream or jet 12 onto the portion 22 of the moving substrate surface 13 of the wheel 14, the melt is chilled into the shape of the ribbon 10 which assumes an inplane curvature defined by the motion of the wheel at the area of impingement 24. The width of the ribbon formed at the melt stream or jet impingement area 24 determines the radius of the inner and outer peripheral edge  $R_i$  and  $R_o$ , respectively, of the edge-wound helical metallic ribbon 10.

The melt stream or jet axis 15 in the plane described may intersect the portion 22 of the moving substrate surface 13 at an angle  $\alpha$  typically between  $30^\circ$  and  $90^\circ$ , with the range  $40^\circ \leq \alpha \leq 70^\circ$  preferred for optimized ribbon geometric uniformity. The structure of the resulting metallic ribbon may be crystalline or glassy. Glassy metallic ribbon may be made from a glassy alloy system by rapid quenching from the melt. Typical examples of glassy alloy systems are Fe-B, Fe-B-C, Fe-B-Si, Fe-Ni-B, Cu-ZR and the like.

It has been empirically found that the edge-wound ribbon most readily forms within certain limits of melt stream or jet velocity and substrate surface velocity. The preferred melt stream or jet velocity should range from about 1 m/s to about 10 m/s. The substrate surface speed preferably ranges from about 12 m/s to about 50 m/s. Precautions must be taken to assure intimate contact between the substrate surface and the cooling ribbon for a sufficient length of time in order to form a suitable helix. One particular method is to roughen the surface of the substrate wheel and thereby prolong ribbon dwell time on the surface of the wheel. Another method is to employ a gas or mechanical type of "hold-down" device which is well known to those skilled in the art.

The ribbon as formed has a substantially uniform cross-section when compared with helical products fabricated by mechanical means of deformation such, for example, as by cambered rolling. The latter products typically have a tapered cross-section wherein the thickness of the ribbon is uniformly reduced towards the outer peripheral edge across the width of the ribbon.

With reference to FIGS. 1 and 1a, the possible orientations of the crucible axis 15 with respect to the moving substrate surface may be defined by an inverted cone with apex at the point of stream axis impingement.

The cone is defined by the inclination and azimuthal angles  $\alpha$  and  $\gamma$ , respectively. Using the projection  $\ell$  as an arbitrary reference marker, the azimuthal angle may have values of  $0 \leq |\gamma| \leq 180^\circ$ . "Backstreaming" occurs when  $|\gamma| > 90^\circ$ , thereby resulting in ribbon 10 formed in the direction of substrate motion and in droplets or a continuous stream formed against the general direction of substrate motion, sometimes resulting in a continuous fiber.

When the melt stream or jet 12 is made to impinge onto a beveled surface 50, that is, a portion of the substrate surface 13 which is modified by shaping it to be integral with and inclined to the remaining portion of the surface 13 of the rotating substrate wheel 14, an edge-wound helical metallic ribbon results and has a nesting angle somewhat less than that of the bevel inclination on the rotating substrate wheel 14. The surface 50 intersects the substrate surface 13 and forms the included obtuse angle  $\beta$  therewith. For example, with reference to FIGS. 2 and 3, the melt jet 12 from crucible 18 is made to impinge upon the beveled surface 50 of the wheel 14 in plane 26 previously described.

The melt stream or jet 12, which is directed onto the moving substrate surface 50, has an axis 15 lying in plane 26 and inclined at  $30^\circ \leq \alpha \leq 90^\circ$  with the surface 50. The plane 26 is defined by the tangent to the rotation of the substrate wheel 14 at the point of melt stream or jet axis 15 intersection 24 and by the normal to the local substrate surface 50 at the same point 24. The range  $40^\circ \leq \alpha \leq 90^\circ$  is preferred for optimized ribbon geometry.

A nested glassy alloy ribbon 54 which is produced has parallel surfaces 56 and 58 inclined away from the central axis 20 of the helical coil.

Alternately, as shown in FIGS. 4 and 5, the melt stream or jet 12 from crucible 18 is made to impinge on a beveled surface 60 formed in the outer portion 62 of the substrate surface 13 of the wheel 14. The surface 60 intersects an extension of the surface 13 of the wheel 14 and forms an included acute angle  $\beta$  therewith. The melt stream of jet 12, which is directed onto the moving substrate surface 60, has a axis 15 lying in plane 26 and inclined at  $30^\circ \leq \alpha \leq 90^\circ$  with the surface 60. The plane 26 is defined by the tangent to the rotation of the substrate wheel 14 at the point of melt stream or jet axis 15 intersection 24 and by the normal to the local substrate surface 60 at the same point 24. The range  $40^\circ \leq \alpha \leq 70^\circ$  is preferred for optimized ribbon geometry. The nested metallic ribbon 64 which is produced has substantially parallel surfaces 66 and 68 which are inclined toward the central axis 20 of the helical coil.

Referring to FIG. 6, the portion 22 of the moving substrate surface 13 on the rotating substrate wheel 14 may be modified in order to form a metallic ribbon 70 with predetermined cutout regions therein. The substrate surface portion 22 is modified by suitable means to contain barrier lines. For example, such lines may be introduced by scribing with a sharp-edged tool or by a silk screening ink application to produce a plurality of lines 72 which define the geometric configuration of the cutout to be made in the inner peripheral portion of the ribbon 70. The lines 72 provide a differential cooling rate between the molten metal cast on the lines 72 and the metal cast on the substrate surface portion 22. The lines 72 made either by the removal of the material from the substrate surface portion 22 or by the application of ink provide a barrier which prevents the cast metal from cooling rapidly in the vicinity thereof. Therefore,

the alloy cast as the result of the contact of the melt and the moving substrate surface portion 22 produces the metallic ribbon. Centrifugal force causes the ribbon 70 to be cast from the wheel after an adequate dwell time required to define the helical shape and causes the portion of the ribbon 70 enclosed by scribe marks to break or flake away and produce individual amorphous flakes or platelets 74. The ribbon 70 is suitable for many types of electromagnetic devices such as, for example, the rotor and stator portions of an electric motor, and applications requiring a pre-defined air gap such as in a ballast or in a linear reactor.

With reference to FIG. 7, there is shown another alternate embodiment of the ribbon 10. In this instance, lines 80 are made on the substrate surface portion 22 of the wheel 14 to form metallic ribbon 82 suitable for use in making the rotor portion of an electric motor. Again, metallic flakes 84 are a by-product. The cutouts are made in the outer peripheral portion of the ribbon 82.

The glassy alloy ribbons 70 and 82 may be employed in AC motor stator for a squirrel cage induction or synchronous motor. The ribbon 82 is suitable for the direct casting of one of more components of an AC motor for squirrel case induction, synchronous with or without amortisseur windings, or hysteresis motors as well as DC or universal motor parts.

Alternately, the barrier imposed by the scribe lines 72 and 80 may be obtained by employing a low thermal conducting, a non-thermal conducting, or a non-wetting medium to delineate the pattern of the flakes 74 and 84.

The flakes or platelets 74 and 84 may be employed in making composites or encapsulated shaped articles made from the flakes.

Referring now to FIG. 8, there is shown a ribbon 90 which embodies cutouts in both the inner and outer peripheral edges of ribbon 90. The ribbon 90 is manufactured in a process which embodies a process very similar to that required for producing ribbons 70 and 82. Metallic flakes are a by-product of the process.

The following examples are illustrative of the teachings of this invention:

#### EXAMPLE I

The substrate was provided by the face of a 7.5 cm diameter OFHC copper wheel as shown in FIG. 1 finished with 400 grit emery paper and rotating at 8500 rpm. Angles  $\alpha$  and  $\gamma$  were set at 50° and 0°, respectively. The angle  $\beta$  was 180°. The Fe<sub>40</sub>Ni<sub>40</sub>B<sub>20</sub> molten alloy jet was at 1200° C. and was formed by extrusion under 60 kPa Ar driving pressure through a 500  $\mu$ m hole in a clear fused quartz crucible. The point of melt jet impingement was at a radius of 3 cm from the axis of the rotating wheel. The resultant product was a glassy alloy helix with average diameter 6 cm, ribbon width 0.9 mm, and ribbon thickness 38  $\mu$ m, as measured by a micrometer.

#### EXAMPLE II

The substrate was provided by the face of a 7.5 cm diameter OFHC copper wheel as shown in FIG. 1 finished with 400 grit emery paper and rotating at a speed resulting in 35 m/s substrate surface speed at point of impingement. Angles  $\alpha$  and  $\gamma$  were set at 70° and 0°, respectively. The angle  $\beta$  was 150°. The Fe<sub>40</sub>Ni<sub>40</sub>B<sub>20</sub> jet 65 was formed by pressurization with 60 kPa Ar and extrusion of the melt through a 500  $\mu$ m round orifice at 1200° C. The resulting helical glassy alloy ribbon sample had

an average diameter equal to that of the wheel at the point of melt jet impingement. The nesting angle of the helix was some 10°-15° less than  $\beta$ .

Although the invention has been described relative to the employment of a free jet stream impinging upon the moving substrate surface to form a dynamic melt puddle from which ribbon is drawn, the apparatus of M. C. Narasimhan, appropriately modified, may be employed as well. The apparatus and process of using it is taught in Belgian Pat. No. 859,694 issued Jan. 2, 1978. In the apparatus of M. C. Narasimhan, the molten alloy jet stream is kept confined to within a full breadth of the slit used in casting.

The invention has been described with the possible embodiment of a continuous pattern of geometric cutouts in either or both of the peripheral portions of the ribbon. However, a continuous pattern of a specific geometry may also be provided within the ribbon itself in order to meet motor performance standards. With reference to FIG. 9, there is shown a portion 100 of a ribbon 104 having walls 102 defining a cut-out in the ribbon which is part of a continuous pattern. The ribbon 104 is manufactured in the same manner as the previous ribbons and employing the same barrier line technique to obtain the continuous pattern. The cut-outs may be of any planar geometrical configuration and are determined by the required motor performance for which the ribbon is employed.

We claim as our invention:

1. A method of casting metallic ribbons in helical form by chill block melt-spinning including the process steps of:

- a. rotating a substrate wheel at a predetermined speed to impart to a casting surface thereon a predetermined surface velocity, said wheel having two major opposed top and bottom surfaces and a peripheral edge surface area interconnecting said major surfaces, said top surface lying substantially normal to the axis of rotation of said wheel and being said casting surface;
- b. positioning a crucible with respect to the moving casting surface with the orientation of the longitudinal axis of said crucible with respect to said casting surface being defined by the inclination angle  $\alpha$  and the azimuthal angle  $\gamma$ ;
- c. forming molten alloy of a predetermined composition in said crucible;
- d. ejecting said molten alloy through an orifice in said crucible to form a melt stream having a preferred velocity, said orifice and said melt stream having axes substantially colinear with the axis of said crucible;
- e. impinging said melt stream onto said moving casting surface; and
- f. rapidly chilling said molten alloy impinging on said moving casting surface to form a continuous length of an edge-wound metallic ribbon having a helical shape, said ribbon having a substantially uniform cross section, a pair of substantially parallel major surfaces, and inner and outer peripheral edges of constant radii, defined by the motion of said casting surface at the locus of impingement of said melt stream thereon.

2. The method of claim 1 wherein the angle  $\alpha$  is from 10° to 90°, the melt stream velocity is from about 1 meter per second to about 10 meters per second, and

the casting surface speed is from about 12 meters per second to about 50 meters per second.

3. The method of claim 2 wherein the angle  $\alpha$  is from  $40^\circ$  to  $70^\circ$ .

4. The method of claim 2 wherein

the molten alloy is a glassy alloy is selected from group consisting of Fe-B, Fe-B-C, Fe-B-Si, Fe-Ni-B, and Cu-Zr.

5. The method of claim 1 wherein

said azimuthal angle has values of  $0 \leq |\gamma| \leq 180^\circ$ .

6. A method of casting nested metallic ribbons in helical form by chill block melt-spinning including the process steps of:

a. providing a substrate wheel, said wheel having two major opposed top and bottom surfaces and a peripheral edge surface area interconnecting said major surfaces, said top surface lying normal to the axis of rotation of said wheel, said wheel having a surface for casting thereon, said casting surface being contiguous with at least said top surface and being the lateral area of the frustum of a right circular cone, the axis of said right circular cone being substantially coincident with said axis of rotation with the apex of said right circular cone being above said top surface;

b. rotating said substrate wheel at a predetermined speed to impart to said casting surface a predetermined surface velocity;

c. positioning a crucible with respect to the moving casting surface with the orientation of the longitudinal axis of said crucible with respect to said casting surface being defined by the inclination angle  $\alpha$  and the azimuthal angle  $\gamma$ ;

d. forming molten alloy of a predetermined composition in said crucible;

e. ejecting said molten alloy through an orifice in said crucible to form a melt stream having a preferred velocity, said orifice and said melt stream having axes substantially colinear with the axis of said crucible;

f. impinging said melt stream onto said moving casting surface; and

g. rapidly chilling said molten alloy impinging on said moving casting surface to form a continuous length of nested metallic ribbon edge-wound in a helical shape, said ribbon having a substantially uniform cross section, a pair of substantially parallel major surfaces, and inner and outer peripheral edges of constant radii defined by the motion of said casting surface at the locus of impingement of said melt stream thereon, said ribbon leaving said moving casting surface with said substantially parallel major surfaces inclined away from the central axis of the helical coil.

7. The method of claim 6 wherein the angle  $\alpha$  is from  $10^\circ$  to  $90^\circ$ , the melt stream velocity is from about 1 meter per second to about 10 meters per second, and the moving casting surface speed is from about 12 meters per second to about 50 meters per second.

8. The method of claim 7 wherein the angle  $\alpha$  is from  $40^\circ$  to  $70^\circ$ .

9. The method of claim 7 wherein the molten alloy is a glassy alloy selected from the group consisting of Fe-B, Fe-B-C, Fe-B-Si, Fe-Ni-B, and Cu-Zr.

10. The method of claim 6 wherein said azimuthal angle has values of  $0 \leq |\gamma| \leq 180^\circ$ .

11. A method of casting nested metallic ribbons in helical form by chill block melt-spinning including the process steps of:

a. providing a substrate wheel, said wheel having two major opposed top and bottom surfaces and a peripheral edge surface area interconnecting said major surfaces, said top surface lying normal to the axis of rotation of said wheel, said wheel having a surface for casting thereon, said casting surface being contiguous with at least said top surface and being the lateral area of the frustum of a right circular cone, the axis of said right circular cone being substantially coincident with said axis of rotation with the apex of said right circular cone being below said top surface;

b. rotating said substrate wheel at a predetermined speed to impart to said casting surface a predetermined surface velocity;

c. positioning a crucible with respect to the moving casting surface with the orientation of the longitudinal axis of said crucible with respect to said casting surface being defined by the inclination angle  $\alpha$  and the azimuthal angle  $\gamma$ ;

d. forming molten alloy of a predetermined composition in said crucible;

e. ejecting said molten alloy through an orifice in said crucible to form a melt stream having a preferred velocity, said orifice and said melt stream having axes substantially colinear with the axis of said crucible;

f. impinging said melt jet stream onto said moving casting surface; and

g. rapidly chilling said molten alloy impinging on said moving casting surface to form a continuous length of nested metallic ribbon edge-wound in a helical shape, said ribbon having a substantially uniform cross section, a pair of substantially parallel major surfaces, and inner and outer peripheral edges of constant radii defined by the motion of said casting surface at the locus of impingement of said melt stream thereon, said ribbon leaving said moving casting surface with said substantially parallel major surfaces inclined toward the central axis of the helical coil.

12. The method of claim 11 wherein the angle  $\alpha$  is from  $10^\circ$  to  $90^\circ$ , the melt stream velocity is from about 1 meter per second to about 10 meters per second, and the moving casting surface speed is from about 12 meters per second to about 50 meters per second.

13. The method of claim 12 wherein the angle  $\alpha$  is from  $40^\circ$  to  $70^\circ$ .

14. The method of claim 12 wherein the molten alloy is a glassy alloy selected from the group consisting of Fe-B, Fe-B-C, Fe-B-Si, Fe-Ni-B, and Cu-Zr.

15. The method of claim 11 wherein the azimuthal angle has values of  $0 \leq |\gamma| \leq 180^\circ$ .

\* \* \* \* \*

UNITED STATES PATENT AND TRADEMARK OFFICE  
CERTIFICATE OF CORRECTION

PATENT NO. : 4,281,706

Page 1 of 3

DATED : August 4, 1981

INVENTOR(S) : Howard H. Liebermann, Peter G. Frischmann &  
George M. Rosenberry, Jr.

It is certified that error appears in the above-identified patent and that said Letters Patent is hereby corrected as shown below:

col. 1, line 56, delete "nest" and substitute therefor  
-- nested --

col. 1, line 59, delete "refabricated" and substitute therefor  
-- prefabricated --

col. 2, line 17, after " $0 \leq |\gamma| \leq 180^\circ$ .", insert, as the beginning  
of a new paragraph, -- The melt stream or jet is caused  
to impinge onto the moving substrate surface at a  
predetermined angle  $\alpha$  therewith. -- (The next two  
sentences beginning with "The axis" at line 17 and "The  
angle" at line 21 belong in the new paragraph).

col. 2, line 22, delete the carat (^) after "of"

col. 2, line 23, delete the carat (^) before " $40^\circ \leq \alpha \leq 70^\circ$ ."

col. 2, line 37, delete "or" and substitute therefor -- of --

col. 3, line 36, delete "he" and substitute therefor -- the --

col. 3, line 40, delete "Cu-ZR" and substitute therefor  
--Cu-Zr --

col. 3, line 55, delete "know" and substitute therefor  
-- known --

UNITED STATES PATENT AND TRADEMARK OFFICE  
CERTIFICATE OF CORRECTION

Page 2 of 3

PATENT NO. : 4,281,706

DATED : August 4, 1981

INVENTOR(S) : Howard H. Liebermann, Peter G. Frischmann, and  
George M. Rosenberry, Jr.

It is certified that error appears in the above-identified patent and that said Letters Patent is hereby corrected as shown below:

col. 4, line 41, delete "of" and substitute therefor -- or --

col. 4, line 42, delete "a" and substitute therefor -- an --

col. 4, line 46, delete "inersecton" and substitute therefor  
-- intersection --

col. 5, line 23, delete "of" (second occurrence) and  
substitute therefor -- or --

col. 5, line 24, delete "case" and insert therefor -- cage --

Claim 4, line 2, delete "the" and insert therefor -- said --

Claim 4, line 2, delete "is" (second occurrence)

Claim 4, line 3, before "group" insert -- the --

UNITED STATES PATENT AND TRADEMARK OFFICE  
CERTIFICATE OF CORRECTION

PATENT NO. : 4,281,706

Page 3 of 3

DATED : August 4, 1981

INVENTOR(S) : Howard H. Liebermann, Peter G. Frischmann, and  
George M. Rosenberry, Jr.

It is certified that error appears in the above-identified patent and that said Letters Patent is hereby  
corrected as shown below:

Claim 6, line 11, delete "frustrum" and insert therefor  
-- frustum --

Claim 11, line 11, delete "frustrum" and insert therefor  
-- frustum --

Signed and Sealed this  
Eighth Day of March 1983

[SEAL]

Attest:

GERALD J. MOSSINGHOFF

Attesting Officer

Commissioner of Patents and Trademarks